# EUROPEAN PATENT APPLICATION

(11) **EP 4 023 781 A1**
(43) Date of publication of application: **06.07.2022**
(21) Application number: 21218233.1
(22) Date of filing: 29.12.2021
(51) Int. Cl.: C22C 5/02, C22C 1/03, C22C 9/00, C22F 1/14

(54) **PROCESS FOR ATTAINING A GOLD ALLOY AND GOLD ALLOY ATTAINED WITH SAID PROCESS**

(30) Priority: 29.12.2020 PL 43650320
(71) Applicant: Tivano Baltic Spólka z Organiczona Odpowiedzialnoscia, 80-747 Gdansk (PL)
(72) Inventor: CERATO, Silverio, 181-00 Prague (CZ)
(74) Representative: Gallo, Luca

(57) **Abstract**

Process for attaining a gold alloy, which comprises a first melting step, in which at least titanium, indium and copper are melted and mixed, attaining a first alloy.

In addition, the process comprises a second melting step, in which at least the first alloy, gold, in a percentage comprised between 4 and 98% by weight, silver, copper and zinc are melted and mixed, attaining a gold alloy with carat weight comprised between 1 and 23.5 carats.

## Description

### Field of application

The present invention regards a process for attaining a gold alloy and a gold alloy attained with said process, according to the preamble of the respective main independent claims.

The present process and gold alloy are generally inserted in the industrial field of production and of working metals and alloys, in particular precious metals and alloys, for goldworking and jewelry.

The process is thus advantageously intended to be used for producing semifinished products made of gold alloys of different carat weights, workable for example via drawing or rolling in order to obtain wire, jewels, necklaces, frames for eyeglasses and other objects made of precious alloy.

### State of the art

In the field of production and working of precious metal alloys, gold alloys are known containing various gold percentages. In particular, it is known that with the increase of the quantity of gold, which is an extremely ductile and malleable metal, the overall hardness and elasticity of the alloy decreases.

There is therefore the particular need in the field to obtain gold alloys, even high-titer, i.e. with high gold content, which simultaneously has sufficient hardness, elasticity and brilliance, while maintaining during working the ductility type of gold.

Generally, gold alloys are attained by means of melting and mixing of specific quantities of gold, silver and copper. In particular, the most common, commercially available jewelry alloys are those containing 75% by weight of gold, i.e. 18 carats, while silver and copper are present in variable percentages depending on the color that one wishes to obtain.

The hardening of the alloy is generally obtained through different methods. For example, the simplest method for increasing the strength is cold deformation. In particular, cold deformation causes the work hardening of the material, leading to an increase of mechanical strength, hardness and wear resistance, to the detriment however of ductility and formability. In addition, a subsequent heating at suitable temperature, according to a heat treatment known in the field with name of annealing, leads to the recrystallization of the metal, considerably reducing the strength thereof.

A second known method is that for solid solution, i.e. with the formation of alloys. In accordance with such known method, the solvent atoms (gold) are substituted with solute atoms (other elements in alloy), introducing deformations in the crystal lattice which increase the quantity of solute and based on the difference between the dimensions of the atoms of the used elements. In this manner, one obtains an increase of the strength and of the hardness, without linked considerable loss of ductility. Based on the values of the atomic radii of gold, silver and copper, it is known that the additions of copper reinforce the gold more than the additions of silver, also in annealing conditions. A further known method provides for subjecting the alloy to thermal treatment. In particular, the alloys gold-silver-copper are single-phase at high temperature and, depending on their carat weight, can become two-phase if cooled slowly. Therefore, the 18-carat gold alloys or gold alloys with lower carat weights are brought to high temperatures (above 650°C for 14-carat alloys and above 550°C for 18-carat alloys) so as to enter into single-phase field, by means of treatment known with the name of solubilization. The solubilized alloys are then tempered, i.e. quickly cooled in water such that there is no phase transformation and the material remains a disordered supersaturated solid solution. In this manner, minimum hardness and maximum ductility are obtained. The alloys thus tempered are then subjected to a treatment known with the name of aging at low temperature, such that there is the precipitation of the second phase in the form of finely dispersed submicroscopic particles so as to form the ordered phases. Alternatively, the transformation from disorder to order can take place accompanied by a considerable increase of the strength and of the hardness. These treatments, known as hardening via aging, cause a considerable increase of the strength and of the hardness of the alloys.

In order to exploit such reinforcement methods or to improve other properties of the alloy, it is known to introduce further elements in the alloy, such as for example zinc, and in much lower quantities also titanium, nickel, silicon, boron, iron and cobalt.

For example, alloys are known containing a small quantity of titanium in order to obtain a greater hardness and wear resistance after the aging treatment. Titanium is in particular used in substitution of ferromagnetic alloying elements, such as for example iron, nickel and cobalt, which are undesired in precious alloys, not only for such magnetic properties but also for the risk of causing allergic reactions.

The above-described gold alloys have in practice shown that they do not lack drawbacks.

A first drawback of the aforesaid gold alloys lies in the fact that in order to amalgamate the titanium in the alloy in a sufficiently uniform manner, it is necessary to provide for at least three melting steps, in which in a first step the titanium is melted with copper, in a second melting step the product of the first melting is melted with other alloying elements (e.g. silver) and finally in a third melting step the gold is added.

In addition, also by executing the aforesaid melting steps, in the above-described gold alloys the titanium can in any case be inserted in an alloy only in small percentages, and therefore the improvement of the hardness of the material after aging remains limited.

A further drawback of the known gold alloys lies in the fact that they require long working times. Indeed, following mechanical working operations for reducing the thickness or the diameter, e.g. by means of rolling or drawing, such alloys must be subjected to annealing in order to eliminate the work hardening and prevent defects and breakage during subsequent working operations. With the presence of the titanium, the alloy work-hardens more quickly, for example after a reduction of diameter or thickness at most by 40-50%, and therefore it is necessary to subject it to more frequent annealing treatments.

A further drawback of the known gold alloys lies in the fact that they also contain high percentages of zinc, which, similar to titanium, leads to the breakage of the product (e.g. of a wire in drawing operations) if the latter is worked for a long time period without annealing.

A further drawback of the known gold alloys lies in the fact that, still due to the presence of titanium and zinc, they are less ductile. Therefore, following the working operations, they have an external surface characterized by high porosity and are provided with "orange peel" appearance. It is therefore necessary to subject the worked alloy to subsequent polishing treatments, which add to the process times and cause the loss of precious material.

### Presentation of the invention

In this situation the problem underlying the present invention is therefore that of overcoming the drawbacks manifested by the abovementioned solutions of known type by providing a process for attaining a gold alloy, which allows uniformly amalgamating the alloy elements without providing for a high number of melts.

A further object of the present invention is to provide a process, which allows decreasing the times of subsequent mechanical working for the attainment of a finished product in gold alloy.

A further object of the present invention is to provide a gold alloy, which has greater hardness than the known gold alloys.

A further object of the present invention is to provide a gold alloy, which simultaneously has good characteristics of ductility, elasticity and brilliance.

A further object of the present invention is to provide a gold alloy, which is strong and durable over time.

A further object of the present invention is to provide a process and a gold alloy, which are simple to attain.

### Brief description of the drawings

The technical characteristics of the present invention, according to the aforesaid objects, can be seen in the content of the below-reported claims and the advantages thereof will be more evident in the following detailed description, made with reference to the enclosed figures, which represent a merely exemplifying and non-limiting embodiment of the invention in which:
- figure 1 shows a graph relative to the increase of hardness over time of a gold alloy embodiment according to the invention during an aging treatment.

### Detailed description of several preferred embodiments

The process for attaining a gold alloy, object of the invention, is advantageously intended for the production of a gold alloy in particular for jewelry and gold working. In addition, the process, object of the invention, is advantageously intended to be employed in the production of semifinished products made of gold alloys of different carat weights, adapted for being mechanically worked by means of processes of reduction of diameter or thickness, e.g. by means of drawing or rolling. More in detail, the gold alloy obtained by means of the process, object of the invention, is advantageously intended to be employed in the production of wires, jewels, necklaces, frames for eyeglasses and other objects made of precious alloy, for which it is highly requested.

In accordance with the idea underlying the present invention, the process comprises a first melting step, in which at least titanium, indium and copper are melted and mixed, attaining a first alloy.

According to the invention, the process also comprises a second melting step, in which at least the first alloy, gold, silver, copper and zinc are melted and mixed. In particular, gold is added in a percentage comprised between 4 and 98% by weight, thus attaining a gold alloy with carat weight comprised between 1 and 23.5 carats.

It was found that the addition of indium in the first alloy has at least a triple effect.

Firstly, the indium advantageously increases the malleability and the ductility of the gold alloy and consequently allows mechanically working it, decreasing the necessary annealing and hence the process times. It is in fact possible to carry out working for reducing diameter or thickness even up to 70-75% before having a considerable work hardening of the gold alloy.

Advantageously, in addition, the increase of malleability and ductility of the gold alloy decreases the porosity thereof following the mechanical working and increases the brilliance thereof, allowing to decrease or prevent expensive polishing treatments. Secondly, the indium allows advantageously increasing the percentage of titanium contained in the gold alloy. In this manner, the gold alloy is stronger both after cold deformation and after aging treatment. Advantageously, in order to increase the hardness of the gold alloy it is sufficient to increase the quantity of the first alloy added in the second melting step.

For example, following an aging treatment, the gold alloy can even reach a hardness of 300 HV after an hour of heating.

Thirdly, the indium advantageously lowers the melting point of the first alloy, since it has a melting point of about 156.6 °C, lower than titanium and copper, which have melting point respectively of 1668 °C and 1085 °C. At the same time, the indium evaporates at a greater temperature (about 2072 °C) with respect to the melting point of such elements and therefore is not dispersed. In addition, the indium advantageously allows a greater mixing of copper and titanium, due to the enlargement of the melting interval.

Preferably, in the first melting step, the titanium is added in a quantity such that the gold alloy contains titanium in a percentage comprised between 0.1 and 1.5% by weight. Preferably, in addition, in the first melting step, the indium is added in a quantity such that the gold alloy contains indium in a percentage comprised between 0.1 and 2% by weight.

Preferably, moreover, the first alloy contains copper in a percentage comprised between 1 and 25% by weight with respect to the weight of the entire gold alloy. Advantageously, if it is necessary to further increase the quantity of copper in the gold, such copper quantity is also added in the second melting step.

Of course, without departing from the protective scope of the invention, such quantities of indium, titanium and copper can be modified by adding more or less quantities of the first alloy in the second melting step.

For example, the first alloy contains titanium in a quantity comprised between 0.4 and 33.3% by weight (with respect to the weight of the first alloy).

In addition, the first alloy advantageously contains indium in a quantity comprised between 0.4 and 44.4 % by weight (with respect to the weight of the first alloy).

In addition, the first alloy advantageously contains copper in a quantity comprised between 22.2 and 94% by weight (with respect to the weight of the first alloy).

In addition, in the second melting step the first alloy is advantageously added in a quantity comprised between 1.2 and 28.5% by weight with respect to the weight of the gold alloy.

Advantageously, the elements in the second melting step are added in a quantity such to bring the gold alloy to the desired carat weight and color.

For example, a quantity of silver greater than that of copper confers to the gold alloy a color similar to green, while a quantity of silver lower than the copper confers a pink or red color to the gold alloy.

Advantageously, in addition, in the second melting step, zinc is added in a percentage equal to or less than 15% by weight, preferably equal to or less than 10% by weight. For example, in an 18-carat gold alloy, i.e. containing 75% by weight of gold, a quantity of zinc of 5% by weight can be used. In particular, the quantity of indium can be decreased by increasing the content of indium and titanium in the first alloy and/or by increasing the content of the first alloy in the second melting step.

Advantageously, in the second melting step, silver is added in a percentage comprised between 1 and 13% by weight.

Advantageously, in addition, in the second melting step, copper is further added in a percentage comprised between 0.8 and 55% by weight.

In accordance with a first embodiment of the invention, the elements contained in the gold alloy are introduced into an alloy usually by means of the first melting step and the second melting step. In this manner, with only two melting steps., it is advantageously possible to lower the production costs and times.

In accordance with a second embodiment of the invention, the process comprises an intermediate melting step, preceding the second melting step, in which at least gold, silver, copper and zinc are melted and mixed, attaining a second alloy. Advantageously, in the second melting step, said first alloy and said second alloy are melted and mixed.

In this manner, even if there are more than two melting steps, it is possible to improve the mixing of the elements contained in the second alloy with each other and with the elements contained in the first alloy.

Of course, without departing from the protective scope of the invention, it is possible to attain multiple intermediate alloys containing two or more melted and mixed elements in further intermediate melting steps preceding the second melting step.

For example, in accordance with a further embodiment, in the second melting step copper and zinc are introduced in brass alloy form. In particular, for the sake of simplicity, the brass alloy is an alloy of known type, e.g. a brass alloy 667, i.e. with a ratio by weight zinc/copper of 667/333, or a brass alloy 815, i.e. with a ratio by weight zinc/copper of 815/185. In particular, the brass alloy 667, with substantially yellow color, can be advantageously used for obtaining a 14-carat green gold alloy (i.e. with a percentage of 58.5% by weight of gold) containing a quantity of silver greater than the quantity of copper. Otherwise, the brass alloy 815, with redder color, can be used for bringing a greater quantity of copper to the gold alloy.

Advantageously, the first melting step is attained in inert atmosphere or under vacuum. Advantageously, in addition, also the second melting step is attained in inert atmosphere or under vacuum.

Also forming the object of the invention is a gold alloy, advantageously attained by means of the above-described process.

In accordance with the idea underlying the present invention, the gold alloy contains at least the following elements: gold, silver, zinc, titanium, indium, copper.

Preferably, the gold alloy has carat weight comprised between 1 and 23.5 carats, preferably between 8 and 22 carats, and contains a percentage by weight of gold comprised between 4 and 98% by weight, preferably comprised between 33 and 92% by weight.

According to the invention, the gold alloy contains titanium in a percentage comprised between 0.1 and 1.5% by weight.

According to the invention, moreover, the gold alloy contains indium in a percentage comprised between 0.1 and 2% by weight.

Advantageously, moreover, the gold alloy contains zinc in a percentage equal to or less than 15% by weight, preferably equal to or less than 10% by weight.

Advantageously, in addition, the gold alloy contains copper in a percentage comprised between 0.8 and 55% by weight.

Advantageously, in addition, the gold alloy contains silver in a percentage comprised between 1 and 13% by weight.

Hereinbelow, an embodiment of the gold alloy is reported according to the above-described method, in particular with 18-carat gold alloy.

In particular, the gold alloy embodiment was obtained by adding, in the first melting step, a quantity of titanium equal to 8.2% by weight, a quantity of indium equal to 9.5% by weight and a quantity of copper equal to 82.3% by weight, for attaining a first alloy. In the second step, a quantity of gold equal to 75% by weight was added in order to obtain a gold alloy with carat weight of 18 carats, a quantity of silver equal to 12% by weight, a quantity of zinc equal to 1.5% by weight and a second quantity of copper equal to 10% by weight. In addition, the first alloy was added, i.e. the product of the first melting step, in a quantity equal to 1.5% by weight.

In particular, the gold alloy according to the embodiment thus obtained is an 18-carat gold alloy with yellow color.

In addition, the gold alloy thus obtained was subjected to an aging treatment which, already after an hour of heating, has conferred to the gold alloy a hardness of 300 HV, as illustrated in figure 1.

The gold alloy, according to the attained embodiment, also has a processability that allows a lower number of annealing operations, with consequent decrease of the production times and costs.

The invention thus conceived therefore attains the pre-established objects.

## Claims

1. Process for attaining a gold alloy, **characterized in that** it comprises the following steps:
- a first melting step, in which at least titanium, indium and copper are melted and mixed, attaining a first alloy;
- a second melting step, in which at least said first alloy, gold, in a percentage comprised between 4 and 98% by weight, silver, copper and zinc are melted and mixed, attaining a gold alloy with carat weight comprised between 1 and 23, 5 carats.

2. Process according to claim 1, **characterized in that** said first melting step is attained in inert atmosphere or under vacuum.

3. Process according to claim 1 or 2, **characterized in that** it comprises an intermediate melting step, before the second melting step, in which at least gold, silver, copper and zinc are melted and mixed, attaining a second alloy; in which in said second melting step, said first alloy and said second alloy are melted and mixed.

4. Process according to any one of the preceding claims, **characterized in that** said first alloy contains copper in a percentage comprised between 1 and 25% by weight with respect to the weight of the entire said gold alloy.

5. Process according to any one of the preceding claims, **characterized in that** in said second melting step, copper and zinc are introduced in brass alloy form.

6. Gold alloy, attained by means of the process according to any one of the claims from 1 to 5, which is **characterized in that** it contains titanium in a percentage comprised between 0.1 and 1.5% by weight and indium in a percentage comprised between 0.1 and 2% by weight.

7. Gold alloy according to claim 6, **characterized in that** it contains zinc in a percentage equal to or less than 15% by weight, preferably equal to or less than 10% by weight.
